

1

2,934,565

## POLYNITROAMINE SALTS

Milton B. Frankel, Pasadena, Calif., assignor to Aerojet-General Corporation, Azusa, Calif., a corporation of Ohio

No Drawing. Application October 29, 1957  
Serial No. 694,695

20 Claims. (Cl. 260—583)

This invention relates to new compositions of matter and a method for their preparation. In particular, this invention relates to bis-inorganic acid salts of gem-dinitro diamines having the general formula:



wherein X is a nitrate or perchlorate radical and A and A' are alkylene radicals which can be the same or different.

Due to their high oxygen content, the gem-dinitro salt compounds of this invention are useful as propellant additives. They also have utility as high explosives and can be used in any conventional explosive missile, projectile, rocket, or the like as the main explosive charge. An example of such a missile is disclosed in United States Patent No. 2,470,162, issued May 17, 1949. One way of using the high explosives in a device such as that disclosed in United States Patent No. 2,470,162 is to pack the crystalline explosive in powder form into the warhead of the missile. Alternatively, the crystals can be first pelletized and then packed. A charge thus prepared is sufficiently insensitive to withstand the shock entailed in the ejection of a shell from a gun barrel or from a rocket launching tube under the pressure developed from ignition of a propellant charge, and can be caused to explode on operation of an impact- or time-fuse mechanism firing a detonating explosive such as lead azide or mercury fulminate.

The compounds of this invention are prepared by reacting a gem-dinitro diisocyanate with dilute nitric or perchloric acid, in accordance with the general reaction scheme set forth below:



wherein X, A and A' are as defined above.

To more clearly illustrate my invention, the following example is presented. It is to be understood, however, that this example is presented merely as a means of illustration and is not intended to limit the scope of the invention in any way.

## EXAMPLE

## Preparation of the nitric acid salt of 3,3-dinitro-1,5-pentane diamine

In a round bottom flask fitted with a reflux condenser, 3,3-dinitro-1,5-pentane diisocyanate was heated with a ten-fold excess of 35% nitric acid on a steam bath for a period of 3 hours. The solution was evaporated to

2

dryness in vacuo leaving a quantitative yield of the bis-nitric acid salt of 3,3-dinitro-1,5-pentane diamine. Upon recrystallization from methanol, the product exhibited a melting point of 151–153° C. The elemental analysis of the product is as follows:

Calculated for  $\text{C}_5\text{H}_{14}\text{N}_6\text{O}_{10}$ : percent C, 18.87; percent H, 4.43; percent N, 26.41. Found: percent C, 19.07; percent H, 4.70; percent N, 26.22.

The explosive power of this compound was calculated 10 to be:

Lead block value, 120 T.N.T.=100  
Ballistic mortar value, 130 T.N.T.=100

As indicated above, a dilute acid is employed for the 15 reaction of the present invention. By dilute acid, as the term is employed herein, is meant an aqueous solution of acid, preferably of from about 30 to about 85% concentration. The reaction of this invention is a vigorous one and I have found that optimum control can 20 be exercised when an acid of about 35% concentration is employed in excess. The excess acid acts as a diluent or solvent and thereby effects moderation of the reaction.

Reaction temperature is not critical in the practice 25 of this invention, the only effect of temperature variation being a corresponding increase or decrease in reaction rate. I have found, however, that elevated reaction temperatures such as those from ambient to about 100° C. result in particularly favorable reaction rates and that 30 the reaction proceeds most efficaciously at steam bath temperature.

The diisocyanates useful as starting materials for the 35 reaction of this invention, such as 3,3-dinitro-1,5-pentane diisocyanate, are prepared by reacting the corresponding diacyl halides, such as 4,4-dinitroheptanedioyl chloride, with an azide of an alkali or alkaline earth metal, such as sodium azide, and subsequently heating under anhydrous conditions to effect rearrangement to the desired diisocyanate, as more fully disclosed in assignee's 40 copending U.S. patent application Serial No. 623,728, filed November 16, 1956.

It will be appreciated that a wide variety of bis-inorganic acid salts of gem-dinitro diamines can be prepared in accordance with the method of my invention.

For example, 4,4-dinitro-1,7-heptane diisocyanate and 45 4,4-dinitro-1,8-octane diisocyanate react with dilute nitric acid to produce the bis-nitric acid salts of the corresponding diamines, namely, 4,4-dinitro-1,7-heptane diamine and 4,4-dinitro-1,8-octane diamine. Similarly, 50 3,3-dinitro-1,5-pentane diisocyanate and 5,5-dinitro-1,9-nonane diisocyanate react with dilute perchloric acid to yield the bis-perchloric acid salts of the corresponding diamines, namely, 3,3-dinitro-1,5-pentane diamine and 5,5-dinitro-1,9-nonane diamine.

It is apparent that any number of my series of novel 55 compounds can be obtained by reacting the appropriate starting materials as taught herein.

This application is a continuation-in-part of my copending U.S. patent application Serial No. 412,103, filed 60 February 23, 1954.

I claim:

1. As new compositions of matter, the bis-inorganic acid salts of gem-dinitro diamines having the general formula:



70 wherein X is a radical selected from the group consisting of nitrate and perchlorate radicals and A and A' are lower alkylene radicals.

2. As new compositions of matter, the bis-nitric acid salts of gem-dinitro diamines having the general formula:



wherein A and A' are lower alkylene radicals.

3. As new compositions of matter, the bis-perchloric acid salts of gem-dinitro diamines having the general formula:



wherein A and A' are lower alkylene radicals.

4. As a new composition of matter, the bis-nitric acid salt of 3,3-dinitro-1,5-pentane diamine having the structural formula:



5. As a new composition of matter, the bis-nitric acid salt of 4,4-dinitro-1,7-heptane diamine having the structural formula:



6. As a new composition of matter, the bis-nitric acid salt of 4,4-dinitro-1,8-octane diamine having the structural formula:



7. As a new composition of matter, the bis-perchloric acid salt of 3,3-dinitro-1,5-pentane diamine having the structural formula:



8. As a new composition of matter, the bis-perchloric acid salt of 5,5-dinitro-1,9-nonane diamine having the structural formula:



9. The method of preparing bis-inorganic acid salts of gem-dinitro diamines having the general formula:



which comprises reacting a gem-dinitro diisocyanate having the general formula:



with a dilute inorganic acid having the general formula HX; wherein X is a radical selected from the group consisting of nitrate and perchlorate radicals and A and A' are lower alkylene radicals.

10. The method of preparing bis-nitric acid salts of gem-dinitro diamines having the general formula:



which comprises reacting a gem-dinitro diisocyanate having the general formula:



with dilute nitric acid; wherein A and A' are lower alkylene radicals.

10. 11. The method of preparing bis-perchloric acid salts of gem-dinitro diamines having the general formula:



which comprises reacting a gem-dinitro diisocyanate having the general formula:



with dilute perchloric acid; wherein A and A' are lower alkylene radicals.

12. The method of preparing the bis-nitric acid salt of 3,3-dinitro-1,5-pentane diamine, which comprises reacting 3,3-dinitro-1,5-pentane diisocyanate with dilute nitric acid.

13. The method of preparing the bis-nitric acid salt of 4,4-dinitro-1,7-heptane diamine which comprises reacting 4,4-dinitro-1,7-heptane diisocyanate with dilute nitric acid.

14. The method of preparing the bis-nitric acid salt of 4,4-dinitro-1,8-octane diamine, which comprises reacting 4,4-dinitro-1,8-octane diisocyanate with dilute nitric acid.

15. The method of claim 9 in which the dilute inorganic acid has a concentration of from about 30% to about 85%.

16. The method of claim 10 in which the dilute nitric acid has a concentration of about 35%.

17. The method of preparing the bis-nitric acid salts of gem-dinitro diamines having the general formula:



which comprises reacting a gem-dinitro diisocyanate having the general formula:



with 35% nitric acid, in the presence of excess dilute nitric acid and at an elevated temperature; wherein A and A' are lower alkylene radicals.

18. The method of preparing the bis-nitric acid salts of gem-dinitro diamines having the general formula:



which comprises reacting a gem-dinitro diisocyanate having the general formula:



with 35% nitric acid, in the presence of dilute nitric acid and at a temperature of about 100° C.; wherein A and A' are lower alkylene radicals.

19. The method of preparing the bis-perchloric acid salt of 3,3-dinitro-1,5-pentane diamine, which comprises reacting 3,3-dinitro-1,5-pentane diisocyanate with dilute perchloric acid.

20. The method of preparing the bis-perchloric acid salt of 5,5-dinitro-1,9-nonane diamine, which comprises reacting 5,5-dinitro-1,9-nonane diisocyanate, with dilute perchloric acid.

## References Cited in the file of this patent

- Feiser et al.: "Organic Chemistry," 1944, D. C. Heath and Co., Boston, page 233.
- 5 Wertheim: "Textbook of Organic Chemistry," 2nd ed., The Blakiston Co., Philadelphia (1946), pp. 308-309.
- Herzog et al.: American Chemical Society-Abstracts of Papers, 118th meeting, 1950, p. 25N.